

[54] BERYLLIUM CONTAINING ROCKET PROPELLANTS PRODUCING MAXIMUM BOOST VELOCITY

[75] Inventors: Arch Scurlock, Arlington; Keith E. Rumbel, Oakton; M. Lee Rice, Alexandria, all of Va.

[73] Assignee: Atlantic Research Corporation, Alexandria, Va.

[22] Filed: Sept. 12, 1963

[21] Appl. No.: 309,369

Related U.S. Application Data

[63] Continuation-in-part of Ser. No. 65,856, Oct. 28, 1960, abandoned.

[52] U.S. Cl. .... 149/19.8, 149/19.3, 149/19.4, 149/19.5, 149/19.6, 149/20, 149/38

[51] Int. Cl. .... C06d 5/06

[58] Field of Search. .... 149/17-20, 149/38-44, 87, 97, 98

[56] References Cited

UNITED STATES PATENTS

|           |        |                |          |
|-----------|--------|----------------|----------|
| 2,970,898 | 2/1961 | Fox            | 149/19 X |
| 2,992,908 | 7/1961 | Hedrick et al. | 149/19   |
| 3,035,948 | 5/1962 | Fox            | 149/19   |
| 3,094,444 | 6/1963 | Hedrick et al. | 149/19   |

Primary Examiner—Benjamin R. Padgett  
Attorney, Agent, or Firm—Martha L. Ross

EXEMPLARY CLAIM

1. In a rocket propellant composition which burns to produce propulsive gases and which consists essentially of a finely-divided, solid, inorganic oxidizer containing combined oxygen which it yields readily for combustion of the fuel components of said composition, and a finely-divided beryllium-containing fuel selected from the group consisting of beryllium, beryllium hydride and mixtures thereof dispersed in an organic fuel matrix comprising at least about 20 per cent by volume of said composition, the improvement in which the oxidizer, the beryllium-containing fuel, and the organic fuel matrix are present in amounts such that the oxidation ratio as defined by the following expression:

$$\text{O/O} + \text{C} + \text{M} \text{ equals about 0.47 to 0.60}$$

wherein O equals the total amount of combined oxygen in the composition, C equals the total amount of carbon, and M equals the amount of beryllium, said O, C and M being expressed in terms of the number of atomic equivalents.

20 Claims, 5 Drawing Figures



Fig. 1



INVENTORS.  
ARCH C. SCURLOCK,  
KEITH E. RUMBLE and  
MILLARD LEE RICE

BY

*Martha L. Ross*  
AGENT

Fig. 2



INVENTORS.  
ARCH C. SCURLOCK,  
KEITH E. RUMBEL and  
MILLARD LEE RICE

BY

*Martha L. Rose*  
AGENT

Fig. 3



INVENTORS.  
ARCH C. SCURLOCK,  
KEITH E. RUMBLE and  
MILLARD LEE RICE

BY

*Martha L. Ross*  
AGENT

Fig. 4



INVENTORS.  
ARCH C. SCURLOCK,  
KEITH E. RUMBLE and  
MILLARD LEE RICE

BY

*Martha L. Rose*  
AGENT

Fig. 5



INVENTORS.

ARCH C. SCURLOCK,  
KEITH E. RUMBLE and  
MILLARD LEE RICE

BY

Martha L. Ross  
AGENT

1

**BERYLLIUM CONTAINING ROCKET  
PROPELLANTS PRODUCING MAXIMUM BOOST  
VELOCITY**

This application is a continuation-in-part of application Ser. No. 65,856 to Arch C. Scurlock, Keith E. Rumbel and Millard Lee Rice, filed Oct. 28, 1960 now abandoned.

This invention relates to new propellant compositions. More specifically, it relates to beryllium-and beryllium hydride-containing propellant compositions of exceedingly high propulsive performance.

The term propellant, as employed herein, refers to compositions comprising an organic fuel binder or matrix containing molecularly combined carbon and hydrogen, an oxidizer, and a particular finely divided metal or metal hydride fuel. When introduced into the combustion chamber of a rocket motor and ignited, such compositions generate high temperature gases, which vent out through the restricted nozzle of the motor at a high velocity to produce thrust.

The parameter generally accepted as indicative of the propulsive performance of a rocket propellant is its specific impulse, which is defined as the lbs. of thrust generated per lb. of propellant per second. Although this characteristic of the propellant is very important as a criterion for evaluating its performance, specific impulse is not the sole factor determining optimum performance in a specific application where the rocket system as a whole, including its inert parts, such as weight of the motor casing and payload, must be considered.

The usual objectives of rocket propulsion are the following:

1. Maximization of altitude and distance attained
2. Minimization of time-to-target
3. Maximization of thrust

Each of these objectives is accomplished by maximizing the boost velocity imparted to the rocket device by combustion of the propellant, the boost velocity being the velocity of the rocket at burn-out less velocity at launching.

We have found that the relationship between boost velocity and the characteristics of the propellant, obtained by applying Newton's second law of motion to the rocket, is defined, for an idealized rocket free of gravitational and drag effects and pressure thrust, by the following equation:

$$\Delta U = I_{sp} g_c \log [1 + \rho/M_i/V_p]$$

where

$\Delta U$  = boost velocity = velocity at burn-out less launching velocity

$M_i$  = mass of inert parts including payload = mass of rocket less mass of propellant

$V_p$  = volume occupied by propellant

$I_{sp}$  = specific impulse of the propellant

$g_c$  = dimensional conversion factor,

32.17 (lb. mass) (ft)/(lb. force) (sec)<sup>2</sup>  $\rho$  = density of propellant

$M_i/V_p$  = mass-to-volume ratio

From this expression of the relationships which determine boost velocity, it will be seen that two additional factors, the density of the propellant and the ratio of the mass of inert parts to the volume of propellant enclosed within the motor, become exceedingly important, particularly at high  $M_i/V_p$  values, as in the

case of boosters and JATO's. In fact, a propellant of high specific impulse but low density can be distinctly undesirable for use at high  $M_i/V_p$  ratios because of a marked drop in boost velocity efficiency.

5 The specific impulse of the propellant is, however, an exceedingly important factor in determining boost velocity at any  $M_i/V_p$  ratio. A propellant having a high specific impulse and producing optimum boost velocity at formulations coincident with optimum specific impulse is of great value to the rocket art, particularly in applications requiring high propulsive performance.

10 The object of this invention is to provide propellant compositions of high specific impulse which produce maximized boost velocities over a wide range of  $M_i/V_p$  ratios.

15 Other objects and advantages will become obvious from the following detailed description and the drawings in which:

20 FIGS. 1 through 4 are graphs comparing performance in terms of boost velocity and specific impulse of propellant formulations containing Be or Be H<sub>2</sub> in different organic binders.

25 FIG. 5 is a graph comparing the performance of several propellants of different specific impulse and density at different ratios of the mass of the inert parts of the rocket vehicle to volume of propellant.

30 Broadly speaking, the invention comprises propellant compositions consisting essentially of a finely divided, solid, inorganic oxidizer and finely-divided beryllium, beryllium hydride or mixtures of the two dispersed in an organic fuel matrix containing molecularly combined carbon and hydrogen, in which the oxidizer and fuel components are present in a particular ratio by weight in terms of the number of atomic equivalents, defined as follows:

$$\text{Oxidation Ratio} = O/O + C + M(v)/(2) = \text{about } 0.47 - 0.60 \text{ preferably } 0.47 - 0.55$$

40 wherein O equals the total amount of oxygen in the propellant composition, C equals the total amount of carbon; M equals the total amount of Be calculated as free metal; and v equals 2, the valence of Be. Thus in the case of the following reaction:



$$\text{the Oxidation Ratio} = 2/2 + 1 + 1(2)/(2) = 0.5$$

45 All molecularly combined oxygen, both in the inorganic oxidizer and in the organic fuel matrix, is included in the determination of total oxygen. Oxygen available for oxidation reaction, as, for example, the active oxygen present in the inorganic oxidizer or in an organic compound, such as a nitrate or nitrite derivative, functions to oxidize molecularly-combined carbon to CO and the metal fuel component to its oxide. Oxygen molecularly bonded to a carbon atom in an organic fuel compound, as, for example, in the case of an ether, alcohol, aldehyde, ketone, ester, amide, etc., though not available for combustion, nevertheless results, by decomposition reaction, in the formation of CO, the desired propulsive gas product. In cases such as organic acids, where decomposition might normally result in the production of CO<sub>2</sub>, under the conditions defined above for the Oxidation Ratio, one of the oxygen atoms preferentially combines with the metal fuel component.

60 When the components are present in a ratio by weight such that the Oxidation Ratio, as defined above,

is 0.5, which will hereinafter be termed as OMO<sub>x</sub> formulation, the oxygen available for combustion of the fuel is stoichiometrically sufficient to oxidize the carbon not already linked to oxygen in the organic fuel to CO and the metal to its oxide. Under such conditions, the molecularly combined hydrogen in the organic fuel compound and in the beryllium hydride, if the latter is used, after ignition of the propellant composition, forms free hydrogen gas, since the molecularly combined carbon and the Be react preferentially with oxygen relative to the hydrogen. The hydrogen gas evolved is heated to a high temperature because of the high exotherm of the oxidizing metal. This, and its low molecular weight make it a very efficient thrust-producing component in the combustion reaction product.

We have discovered that propellant formulations containing finely divided Be, Be H<sub>2</sub> or mixtures of the two as highly exothermic fuel components, have maximum specific impulse and impart optimum boost velocity to the rocket system when the ratio of oxygen to fuel (organic and metal) is at OMO<sub>x</sub> or closely approaches OMO<sub>x</sub>, namely where the Oxidation Ratio equals about 0.47 to 0.60 and, in some applications, preferably about 0.47 to 0.55. The Be fuel, in such formulations, has the additional, highly advantageous characteristic of forming a highly stable refractory oxide which does not decompose or vaporize to any substantial degree after formation, either under the high temperature, high pressure conditions prevailing in the combustion chamber or during venting of the combustion gases out of the nozzle. Dissociation and/or vaporization of the metal oxide are undesirable since such phenomena absorb substantial amounts of heat energy, thereby reducing the temperature and pressure of the low molecular weight thrust-producing combustion gases.

These findings are graphically illustrated by the data summarized on the graphs of FIGS. 1, 2, 3, and 4. FIG. 1 shows the curves for specific impulse and boost velocity of formulations comprising Be and ammonium perchlorate in a polyurethane fuel binder. This binder comprises a mixture of 56.6 percent P-2 prepolymer (polypropylene glycol prepolymerized with an excess of tolylene diisocyanate; molecular weight 2025), 13.7 percent castor oil, 28.1 percent dioctyl azelate, 0.15 percent ferric acetyl acetonate, 1 percent lecithin, and 0.7 percent phenyl- $\beta$ -naphthylamine. FIGS. 2 and 3 summarize similar data for formulations employing a double base binder consisting of nitrocellulose gelled with a mixture of nitroglycerine and dibutyl phthalate and a binder comprising polyvinyl chloride plasticized with dioctyl adipate, respectively. FIG. 4 compares the specific impulse and boost velocity of formulations comprising a double base binder consisting of nitrocellulose and trimethylolethanetrinitrate, ammonium perchlorate and beryllium hydride. All data were determined assuming shifting chemical equilibrium. The boost velocity was determined at an M<sub>i</sub>/V<sub>p</sub> ratio of 60 lbs/cu ft in FIGS. 1 and 2, and at an M<sub>i</sub>/V<sub>p</sub> ratio of 25 lbs/cu ft in FIGS. 3 and 4. It will be noted that in all of the formulations, the highest specific impulse and the highest boost velocity are obtained within the Oxidation Ratio range of 0.47 to 0.60 with the peak at or very close to OMO<sub>x</sub>. Both the specific impulse and the boost velocity are very high, in the case of the beryllium-polyurethane composition the maxima being 283 lb-

sec/lb and 9,160 ft/sec respectively, in the case of the beryllium-double base composition 280 lb-sec/lb and 9,185 ft/sec, in the case of the plasticized beryllium-polyvinyl chloride formulation 280.1 lb-sec/lb and 14,840 ft/sec, and in the case of the beryllium hydride-double base formulation 312.2 lb-sec/lb and 14,375 ft/sec.

It will further be noted that the curves for maximum boost velocity conform very closely to those for maximum specific impulse, a characteristic which is highly advantageous since such propellant compositions provide consistently high performance over a broad range of M<sub>i</sub>/V<sub>p</sub> ratios.

FIG. 4 compares the performance of a number of propellant compositions relative to a reference propellant, on propulsion of an idealized rocket vehicle, i.e., one in which the effects of drag, gravity, and pressure thrust are neglected, exhausting to 14.7 psi from a combustion chamber pressure of 1,000 psi. It will be noted that the beryllium-and beryllium hydride-containing propellents show consistently high performance in terms of boost velocity relative to that of the reference propellant, whereas the very dense Zr-containing propellant, while exceedingly effective at high M<sub>i</sub>/V<sub>p</sub> ratios, drops rather sharply in performance at low ratios and the low-density propellant comprising a mixture of liquid oxygen and hydrazine, while performing well at low M<sub>i</sub>/V<sub>p</sub> ratios, drops sharply in boost velocity performance at high ratios.

As aforementioned, the organic fuel matrix can be any suitable organic compound or mixture of organic compounds which contains molecularly combined carbon and hydrogen, so that at OMO<sub>x</sub> stoichiometry it burns and/or decomposes to produce CO and free hydrogen gas. It can be "inert", the term "inert" as used herein meaning a compound which requires an external source of oxygen, namely the solid, inorganic oxidizer, for combustion. Illustrative of suitable organic matrix compositions are the various solid polymeric binders, such as polyether, polysulfides, polyurethanes, butadiene-acrylic acid and -methacrylic acid copolymers cross-linked with an epoxy, alkyd polyesters, polyamides, cellulose esters, e.g., ethyl cellulose, polyvinyl chloride, asphalt, and the like. The oxygen linked to carbon in a variety of such inert fuel binders produces CO by decomposition reaction.

Many of the solid polymeric binders preferably include high-boiling, organic, liquid plasticizers to improve physical properties and processing of the propellant composition. Any of the numerous organic plasticizers known in the art and compatible with the propellant composition can be employed. Illustrative examples of suitable organic plasticizers include sebacates such as dibutyl sebacate and dioctyl sebacate; phthalates, such as dibutyl phthalate and dioctyl phthalate; adipates, such as dioctyl adipate; glycol esters of higher fatty acids, and the like.

The organic fuel matrix can also comprise an active organic compound, a mixture of such compounds, or a mixture of such a compound with an inert organic compound, such as an inert organic plasticizer, the term "active" compound as employed herein meaning a compound which contains molecularly combined oxygen available for combustion of other components of the molecule, such as carbon. Examples of active organic fuel compounds include those containing nitroso, nitro, nitrite, and nitrate radicals, such as cellulose ni-

trate, nitroglycerine, trimethylolethanetrinitrate, diethyleneglycoldinitrate and the like.

The foregoing description has dealt mainly with solid propellant compositions in which the organic fuel binder is a solid. The invention can also be employed in semi-solid, composite monopropellant systems. Such compositions are thixotropic, cohesive, shape-retentive compositions which can be extruded under moderate pressures into the combustion chamber of a rocket, where they form continuously advancing columns which burn on the exposed surface. In accordance with this invention, such plastic monopropellant compositions comprise a stable dispersion of a finely divided, insoluble oxidizer and the finely-divided Be, Be H<sub>2</sub> or mixtures of the two in a continuous matrix of any suitable high-boiling organic liquid fuel containing molecularly combined carbon and hydrogen. Illustrative of suitable liquid fuels are hydrocarbons, such as triethyl benzene, liquid polyisobutylene, and the like; organic esters, such as dimethyl maleate, dibutyl oxalate, dibutyl phthalate and nitroglycerine; alcohols, such as benzyl alcohol and triethylene glycol; ethers, such as methyl β-naphthyl ether; and many others.

Any solid inorganic oxidizer can be employed which yields oxygen readily for combustion of the metal fuel component and the organic matrix, where the latter contains no oxygen or insufficient oxygen for CO stoichiometry. Such oxidizers include the inorganic oxidizer salts, such as NH<sub>4</sub>, K, Na, and Li perchlorates and nitrates, metal peroxides, such as CaO<sub>2</sub>, BaO<sub>2</sub>, and Na<sub>2</sub>O<sub>2</sub>, nitronium perchlorate, hydrazine nitrate, hydrazine nitroform and the like, the salts being preferred.

Where the organic fuel matrix contains molecularly combined oxygen available in at least the stoichiometric amount required for oxidation and/or decomposition of the molecularly combined carbon component to CO, no inorganic oxidizer need be provided for its combustion. If such combined oxygen is present in amounts greater than that required for such stoichiometry, the amount in excess preferentially oxidizes the powdered metal component rather than the molecularly combined hydrogen and thus can replace a portion of the inorganic oxidizer which would normally be required to oxidize the metal.

The organic fuel matrix, whether it be inert or active, solid or liquid, as aforescribed, must comprise at least about 20 percent, in some cases preferably at least 30 percent, by volume of the propellant composition. This is essential both to provide for generation of an adequate amount of low molecular weight combustion gases requisite for effective propulsion and for processing of a cohesive propellant composition having good physical properties.

The amounts of Be, Be H<sub>2</sub> or mixtures of the two and solid, inorganic oxidizer employed must be such as to produce, with the particular kind and concentration of organic matrix, an Oxidation Ratio within the specified range of about 0.47 to 0.60. This can readily be calculated by use of the equation given above for determination of this expression.

The following examples are illustrative of propellant formulations within the scope of the invention:

#### Example 1

A solid perforated, internally-burning, propellant grain, 6 inches in diameter and weighing 10 lbs. was

prepared by mixing the following components and then curing the mixture to form a polyurethane binder by reaction of the P-2 prepolymer with the castor oil polyol.

|    | Weight %                         |
|----|----------------------------------|
| 10 | *P-2 prepolymer                  |
|    | Castor Oil                       |
|    | Diethyl azelate                  |
|    | Ferric acetyl acetonate          |
|    | Lecithin                         |
|    | Phenyl-β-naphthylamine           |
|    | Be                               |
|    | NH <sub>4</sub> ClO <sub>4</sub> |

15 \*P-2 prepolymer: polypropylene glycol prepolymerized with an excess of tolylene diisocyanate. Molecular weight 2025.

The burning rate of this OMOx formulation in the motor was 0.217 in/sec at a combustion chamber pressure of 1,070 psi.

#### Example 2

A solid propellant grain was made from a composition comprising:

|    | Weight %                                                                  |
|----|---------------------------------------------------------------------------|
| 30 | Nitrocellulose (12.6%N)<br>(Spheres about 15 microns<br>in diameter)      |
|    | 23.88                                                                     |
|    | Nitroglycerine/dibutyl phthalate 75/25 containing 1% 2-nitrodiphenylamine |
|    | 28.08                                                                     |
|    | Dibutyl sebacate                                                          |
|    | 2-Nitrodiphenylamine                                                      |
|    | Be                                                                        |
|    | NH <sub>4</sub> ClO <sub>4</sub>                                          |

The propellant was prepared by the plastisol method. The components were mixed at room temperature and the mixture was then placed in a mold and cured by heating to dissolve the nitrocellulose in the nitroglycerine, dibutyl phthalate, and dibutyl sebacate plasticizers. The Oxidation Ratio of this composition was 0.507. Burning rate of the grain in the motor was 0.525 in/sec at a pressure of 1,055 psi.

#### Example 3

A solid propellant grain was made from a composition comprising:

|    | Weight %                                                             |
|----|----------------------------------------------------------------------|
| 55 | Nitrocellulose (12.6%N)<br>(Spheres about 15 microns<br>in diameter) |
|    | 20.0                                                                 |
|    | Nitroglycerine                                                       |
|    | 9.0                                                                  |
|    | Dibutyl phthalate                                                    |
|    | 35.1                                                                 |
|    | NH <sub>4</sub> ClO <sub>4</sub>                                     |
|    | 14.9                                                                 |

The propellant was prepared by the plastisol method. The components were mixed at room temperature and the mixture was then placed in a mold and cured by heating to dissolve the nitrocellulose in the nitroglycerine and dibutyl phthalate plasticizers. The Oxidation Ratio of this composition was OMOx. Burning rate of the grain at 70°F and 1000 psi was 0.57 in/sec.

#### Example 4

A solid propellant grain was made from a composition comprising:

|                           | Weight % |
|---------------------------|----------|
| $\text{NH}_4\text{ClO}_4$ | 67.49    |
| Dibutyl sebacate          | 10.80    |
| Polyvinyl chloride        | 7.20     |
| Be                        | 14.51    |

The propellant was prepared according to the plastisol method by blending the components at room temperature, pouring the mixture into a mold and heating to dissolve the PVC in the liquid plasticizer, thereby forming a rigid gel. The Oxidation Ratio was  $\text{OMOx}$ . Burning rate at  $70^\circ\text{F}$  and 1,000 psi was 0.49 in/sec.

#### Example 5

A solid propellant grain was made from a composition comprising:

|                                                                      | Weight % |
|----------------------------------------------------------------------|----------|
| Nitrocellulose (12.6%N)<br>(Spheres about 15 microns<br>in diameter) | 18.90    |
| Trimethylolethanetrinitrate                                          | 48.80    |
| Diethyleneglycoldinitrate                                            | 8.20     |
| Ethyl centralite                                                     | 1.20     |
| Alkyl aryl polyether alcohol<br>wetting agent                        | 0.20     |
| Be $\text{H}_2$                                                      | 14.70    |
| $\text{NH}_4\text{ClO}_4$                                            | 8.00     |

The propellant was prepared by the plastisol method. The components were mixed at room temperatures and the mixture was then placed in a mold and cured by heating to dissolve the nitrocellulose in the trimethylolethanetrinitrate and diethyleneglycoldinitrate plasticizers. The Oxidation Ratio of this formulation was  $\text{OMOx}$ . Burning rate of the grain in the motor was 0.500 in/sec at a pressure of 1,055 psia and 0.860 in/sec at a pressure of 1,850 psia.

#### Example 6

A solid propellant grain was made from the following composition:

|                                                                      | Weight % |
|----------------------------------------------------------------------|----------|
| Nitrocellulose (12.6%N)<br>(Spheres about 15 microns<br>in diameter) | 13.47    |
| Trimethylolethanetrinitrate                                          | 34.71    |
| Diethyleneglycoldinitrate                                            | 5.83     |
| Ethyl centralite                                                     | 0.82     |
| Alkyl aryl polyether<br>alcohol wetting agent                        | 0.17     |
| Be $\text{H}_2$                                                      | 11.10    |
| Be                                                                   | 6.20     |
| $\text{NH}_4\text{ClO}_4$                                            | 27.70    |

The propellant was prepared by the plastisol method as described in Example 5. The Oxidation Ratio of the formulation was  $\text{OMOx}$ . Burning rate of the grain in the motor was 0.520 in/sec at a pressure of 580 psia and 0.560 in/sec at a pressure of 850 psia.

Although this invention has been described with reference to illustrative embodiments thereof, it will be apparent to those skilled in the art that the principles of this invention can be embodied in other forms but within the scope of the claims.

We claim:

1. In a rocket propellant composition which burns to produce propulsive gases and which consists essentially of a finely-divided, solid, inorganic oxidizer containing

combined oxygen which it yields readily for combustion of the fuel components of said composition, and a finely-divided beryllium-containing fuel selected from the group consisting of beryllium, beryllium hydride

5 and mixtures thereof dispersed in an organic fuel matrix comprising at least about 20 per cent by volume of said composition, the improvement in which the oxidizer, the beryllium-containing fuel, and organic fuel matrix are present in amounts such that the Oxidation

10 Ratio as defined by the following expression:

$$\text{O}/\text{O} + \text{C} + \text{M} \text{ equals about } 0.47 \text{ to } 0.60$$

wherein O equals the total amount of combined oxygen in the composition, C equals the total amount of carbon, and M equals the amount of beryllium, said O, C and M being expressed in terms of the number of atomic equivalents.

2. The propellant composition of claim 1 in which the organic fuel matrix comprises at least about 30% by 20 volume of the composition.

3. The propellant composition of claim 1 in which the beryllium-containing fuel is beryllium.

4. The propellant composition of claim 1 in which the expression:  $\text{O}/\text{O} + \text{C} + \text{M}$  equals about 0.47 to 0.55.

25 5. The propellant composition of claim 1 in which the Oxidation Ratio equals about 0.5.

6. The propellant composition of claim 1 in which the beryllium-containing fuel is beryllium hydride.

7. The propellant composition of claim 1 in which the beryllium-containing fuel is a mixture of beryllium and beryllium hydride.

30 8. In a rocket propellant composition which burns to produce propulsive gases and which consists essentially of a finely-divided, solid, inorganic oxidizing salt containing combined oxygen which it yields readily for combustion of the fuel components of said composition, and a finely-divided beryllium-containing fuel selected from the group consisting of beryllium, beryllium hydride, and mixtures thereof dispersed in a fuel matrix consisting essentially of an organic polymer, said fuel matrix comprising at least 20 percent by volume of said composition, the improvement in which the oxidizer, the beryllium-containing fuel, and the fuel

35 matrix are present in amounts such that the expression of the Oxidation Ratio  $\text{O}/\text{O} + \text{C} + \text{M}$  equals about 0.47 to 0.60, wherein O equals the total amount of combined oxygen in the composition, C equals the total amount of carbon, and M equals the amount of beryllium, said O, C, and M being expressed in terms of the number of atomic equivalents.

40 9. The propellant composition of claim 8 in which the fuel matrix comprises at least 30 percent by volume of the composition.

55 10. The propellant composition of claim 8 in which the expression  $\text{O}/\text{O} + \text{C} + \text{M}$  equals about 0.47 to 0.55.

11. The propellant composition of claim 10 in which the expression  $\text{O}/\text{O} + \text{C} + \text{M}$  equals about 0.5.

60 12. The propellant composition of claim 10 wherein said beryllium-containing fuel is beryllium.

13. The propellant composition of claim 12 wherein said fuel matrix contains nitrocellulose.

65 14. The propellant composition of claim 12 wherein said oxidizing salt is ammonium perchlorate.

15. The propellant composition of claim 10 in which said beryllium-containing fuel is beryllium hydride.

16. The propellant composition of claim 15 in which said fuel matrix contains nitrocellulose.
17. The propellant composition of claim 15 in which said oxidizing salt is ammonium perchlorate.
18. The propellant composition of claim 10 in which said beryllium containing fuel is a mixture of beryllium

and beryllium hydride.

19. The propellant composition of claim 18 in which said fuel matrix contains nitrocellulose.
20. The propellant composition of claim 18 in which said oxidizing salt is ammonium perchlorate.

\* \* \* \* \*

10

15

20

25

30

35

40

45

50

55

60

65